

Patented Mar. 2, 1926.

1,575,167

# UNITED STATES PATENT OFFICE.

KANESHI KAWAKAMI, OF HONGO-KU, TOKYO, JAPAN.

## PROCESS FOR MANUFACTURING A LEAD ACCUMULATOR.

No Drawing.

Application filed October 3, 1921. Serial No. 505,177.

To all whom it may concern:

Be it known that I, KANESHI KAWAKAMI, a subject of the Emperor of Japan, residing at No. 3 Komagome-Akebono-Cho, Hongo-Ku, Tokyo, Japan, have invented a new and useful Process for Manufacturing a Lead Accumulator, of which the following is a specification.

This invention relates to a process for manufacturing a porous lead for lead accumulators or of a porous lead alloy from a lead alloy. For example, an alloy of lead and potassium, lead and magnesium, lead, potassium and mercury, lead, magnesium and calcium or its compounds, lead, antimony and mercury, and of other alloy of lead with one or more metals in the magnesium group, the alkali group, the alkaline earth group, the arsenic group, the tin group, or the aluminum group. The method of producing such porosity in the lead or alloy consists in driving out a partly melted portion of the alloy by mechanical treatment, such as treatment in a centrifugal separator, while heating the said alloy to a temperature below its melting point and while keeping the same at that temperature. The objects of this invention are, first, to obtain a lead accumulator of high electrical efficiency and of long life; second, to obtain the same of high weight efficiency.

In carrying out the invention, I take as an example, an alloy, in a shape of a plate, ribbon, rod, or like desired shape, of a composition consisting of 93 per cent of lead, 1 per cent of mercury and 6 per cent of antimony, respectively, in weight. A frame or grid, consisting of lead, or of an alloy of 99 per cent of lead and 1 per cent of mercury, in which the aforesaid alloy is cast, or fused therein, may be taken instead of the foregoing plate of the alloy. Such plate of the alloy is heated, in a centrifugal separator, for 20 to 30 minutes by means of an electric current to below its melting point, that is to say, to about a temperature 300° C., until the said plate is uniformly heated, and is then submitted to mechanical treatment, such as treatment in a centrifugal separator, keeping the same at said temperature. After a few minutes of such treatment a melted alloy, constituting a eutectic or eutectics, contained therein, consisting of 13 per cent of lead and 87 per cent of antimony in weight, is driven off and the remaining product is a porous metallic body

consisting of about 97.8 per cent of lead, about 1.8 per cent of mercury and about 0.4 per cent of antimony in weight. When the framed alloy plate is treated in the like manner, I have found that no change in structure of the frame or grid of lead, or of an alloy of lead and mercury, takes place. The said porous product thus obtained may be used as a battery plate, in that condition according to its shape, or may be set in a frame or grid, by being cast or fused therein, and submitted to treatment and formation such as commonly applied heretofore to an ordinary electric accumulator plate.

In carrying out this invention the following alloys, may also be used instead of the aforesaid alloy, and whose proportion of constituents, temperature applicable to them, and proportion of constituents constituting the eutectics driven out, and of the finished products are respectively as follows:

Alloy of 99.2% of lead and 0.8% of magnesium in weight, application of temperature about 280° C., constitution of eutectic 97.1% of lead and 2.9% of magnesium, finished product of about 100% of lead;

Alloy of 99.1% of lead, 0.8% of magnesium and 0.1% of calcium or its compound, application of temperature about 280° C., constitution of eutectic 97% of lead, about 2.9% of magnesium and about 0.1% of calcium, or its compound, finished product of about 100% of lead;

Alloy of 99.4% of lead and 0.6% of potassium, application of temperature about 300° C., constitution of eutectic about 98.2% of lead and about 1.8% of potassium, finished product of about 100% of lead.

The proportions of the constituents for the alloy and the temperature to be applied, may be varied slightly, so as to obtain finished porous products of a fine, or of a coarse structure, according to requirements in use.

In the separating process of the given example, where the initial alloyed plate contained lead and antimony, very thin films of antimony are apt to remain on the inner surfaces of the finished porous product, but, if mercury was added in the said lead-antimony alloy, then the retaining action of the antimony films is considerably reduced. The porous metals thus prepared are particularly suitable as battery plates.

The effect of the mercury contained in the lead alloy is to increase considerably the

mechanical strength of the alloy, and from 0.5 to 5.0 per cent of mercury is very particularly advantageous in this respect. Moreover, in the aforesaid separating process, this alloy used for the frame or grid, etc., causes no change in its structure, and is in this respect like pure lead; but its strength is much higher than the latter.

The existence of mercury in the grain of 10 the lead as a solid solution causes an increase in the strength of the porous lead alloy. This is not only advantageous for the battery plate from a mechanical point of view, but also advantageous from an electro- 15 chemical point of view in that the mercury contained in the lead battery plate suppresses local discharge and other detrimental actions.

Besides the foregoing actual example, it is 20 possible to obtain a porous lead, or a porous lead alloy, from binary or plural elements, consisting of lead with a metal, or metals of the magnesium group, the alkali group, the tin group, the arsenic group, the alkaline 25 earth group and the aluminium group, by the same method as described above.

In the method of forming the porous body of lead, as traces of every constituent may 30 remain in the lead body after the alloy constituting the eutectic is driven off, its effect varies according to the different alloy employed; thus, when it is desired to entirely 35 exclude antimony, the porous lead body, produced by the present process, may be formed with an alloy of lead and magnesium, or potassium, and it is commonly known that magnesium or potassium remaining therein, is especially when used with a sulphuric com- 40 pound, that is to say, a considerable advan-

tage may be obtained by employing magnesium or potassium in such porous lead.

The battery plates made in accordance with the process herein described have an extremely large capacity as compared with 45 those manufactured by the ordinary methods. Moreover, the adhesion between the frames or grids, or conducting members and the finished porous products, or active materials, and also the cohesion between the 50 active material particles are excellent and, further, the local discharge and other detrimental actions are suppressed. Therefore, the electric accumulator constructed with such porous plates has an extremely high 55 weight efficiency, high electrical efficiency and long life, by virtue of the toughness and high qualities of the active materials.

So far as it does not depart from the essential idea of this invention, similar or 60 equivalent steps or stages in the procedures of the process as described, which can bring about the same effect, may be carried out without departing from the spirit of this invention. 65

What I claim is:—

1. A battery element comprising a solid solution of a small percentage of mercury in a large percentage of lead alloyed with a small percentage of antimony, in the form 70 of a porous plate.

2. A battery element comprising a solid solution of 97.8% of lead, 1.8% of mercury in solid solution with the lead, and .4% of antimony alloyed therewith, in the form of 75 a porous plate.

In witness whereof I have hereunto set my hand.

KANESHI KAWAKAMI.